

## UNITED STATES PATENT OFFICE

2,320,108

## COLOR PHOTOGRAPHY

Alan Gilbert Tull, London, England, assignor to  
 Latta Syndicate Limited, London, England, a  
 British company

No Drawing. Application December 17, 1940, Se-  
 rial No. 370,557. In Great Britain February 22,  
 1940

4 Claims. (Cl. 95—2)

This invention relates to the production of color photographs and is concerned primarily with a method of producing a multi-color transparency or reflection print such as a paper print. The invention also embraces a form of multi-layer photographic material for the production of such color photographs.

One object of the invention is a simple and effective method of processing a multi-layer or multi-strata material to produce differently colored images at different depths of the emulsion or in the different layers.

A further object of the invention is to provide a simple method of toning the residual halide of a photographic emulsion to form a reversed colored image without first removing the developed latent image in said emulsion and without converting the said halide to silver as a preliminary stage.

A further object of the invention is to improve or modify the color of an image produced by chemical toning processes.

Still further objects relate to a multi-layer photographic material which is designed for the production of a reflection print and embodies a layer which is initially transparent and can later be converted to an opaque white layer, and to a material embodying a stripping layer whereby the colored image layers can be transferred to a new support.

The present invention may be applied to a two-color process and for this purpose a material is preferably utilised having a support of transparent material such as Celluloid on which is coated first a photographic silver halide emulsion layer which is either non-color sensitised and accordingly blue sensitive or it may be sensitised for green as well so that the layer is blue-green sensitive. Onto this emulsion layer is coated a red or red-yellow sensitive emulsion layer. As this layer remains blue sensitive, a yellow filter layer is preferably interposed between the two emulsion layers to prevent access of blue light to the red-sensitive layer when exposure is made through the support, or if, as is probable, the red sensitive layer is also strongly green sensitive, an orange or red filter layer is interposed instead of yellow.

Such material is exposed in a camera through the support and is processed as described hereinafter either to a negative or to a positive which is a natural color reproduction of the original subject, or it may be used as a copy material for reproducing colored records or color separation records; such a colored record might

have been made, for instance, on similar-type material. In the case of production of a positive directly on the exposure material, the processed material may be applied to a paper support to form a reflection print. However, the original exposure being normally made through the support, the finished positive would have to be viewed from the emulsion side to obtain correct lateral rendering and if the material were applied to a paper base the original support, generally Celluloid, would come between the colored image layers and the paper and would interfere with the correct viewing of the colored images.

15 The present invention therefore includes the provision of a layer between the original support and the emulsion layers, which is initially transparent and can be or is rendered opaque white or opalescent during the processing, forming a reflective layer enabling the colored images to be viewed by reflection. Such a processed material could be applied to a paper or card support for convenience and the paper behind the white layer will tend to improve the reflective properties of the white layer.

20 Such a layer may consist of gelatine containing a proportion of colloidal zinc hydroxide giving a layer which is highly transparent. During the processing the material is inserted in a bath which converts the zinc hydroxide to an insoluble white zinc salt such as zinc carbonate or zinc ferrocyanide.

25 As an alternative to the use of such a layer a stripping layer could be used in the same position, enabling the colored image layers to be removed from the original support and transferred to a new support. Such a layer may consist of soft gelatine, wax, resin or the like, and is so designed that the processing may be carried 30 through to completion on the original support while further soaking, for instance in warm water, enables the colored image layers to be stripped off.

35 If it is desired to produce a color transparency such a stripping or reflective layer need not be used or provided. If the material is processed to a positive natural color record, the colored picture may be used directly for projection for instance in the form of a motion-picture film. It may however be used for the production of 40 duplicate copies on a material of the same general type.

45 It may be preferable however to employ a negative-positive technique if the production of 50 duplicate copies is required. In this procedure

the exposure material is processed to a negative without a reversal stage and may be in colors complementary to the layer sensitivity or otherwise, and positive copies in natural colors are printed therefrom, the procedure in this case again not involving a reversal stage.

In the processing of such a material in accordance with the present invention the basic feature is the conversion of silver salt images, which may be derived from the latent image as in non-reversal or negative-positive processing or from the residual halide after development of the latent image, as in reversal processing, into colored metallic salts or compounds forming the colored images.

The images in the two layers must be processed to different colors and it has been discovered that a conversion bath containing components for the production of a plurality of different colored metallic salts will under suitable conditions deposit the different salts predominantly at different depths of the emulsion layers, thus enabling one color to be deposited primarily in the surface layer and another color predominantly below.

This is particularly noticeable for instance in a reversal technique in which the first developed silver is not removed and a bath containing a ferric salt and a uranium salt and a carefully controlled quantity of potassium bromide is used. If superposed image layers or strata containing silver ferrocyanide produced from the residual halide are treated in such a bath, a Prussian blue image is formed exclusively in the surface stratum or layer while there is a red image of uranyl ferrocyanide below that, enabling a natural color picture to be produced on the type of material specifically described above.

In one method of processing such a two layer material, after exposure, for instance in a camera, to produce a natural color picture, the first stage is the development of the latent images in a silver solvent developer such as the following:

*Formula I*

|                         |      |      |
|-------------------------|------|------|
| Metol                   | gm.  | 0.5  |
| Hydroquinone            | gms. | 4.0  |
| Sodium sulphite anhyd.  | gms. | 25.0 |
| Sodium carbonate anhyd. | gms. | 17.5 |
| Potassium bromide       | gms. | 2.5  |
| Potassium thiocyanate   | gms. | 4.5  |
| Water to                | ccs. | 500  |

The next step is the conversion of the residual halide in both layers into silver ferrocyanide. This may be done by methods well known in the art, which involve the removal of the developed latent image silver by reagents which have no effect on the residual halide, followed by development of the latent image to silver and bleaching in an oxidising bath to form silver ferrocyanide ferrocyanide. This is, broadly speaking the only known method of converting the halide into silver ferrocyanide but it has been discovered that the conversion can be more simply effected directly in the presence of a reagent which reverses the relative solubility of the halide and ferrocyanide, that is to say a reagent in which the ferrocyanide is less soluble than the halide. Such a reagent is thiourea, although ammonia, potassium thiocyanate, thioacetamide, thiosinamine or cysteine could be used.

The latter method has been found advantageous moreover because the presence of the first developed silver appears to facilitate the regular performance of the subsequent toning operations

and this method is preferably employed. The following conversion bath has been found to be satisfactory for this purpose:

|   |                                     |     |
|---|-------------------------------------|-----|
| 5 | <i>Formula II</i>                   | cc. |
|   | 5% thiourea solution                | 10  |
|   | 10% potassium ferrocyanide solution | 40  |
|   | Water to                            | 150 |

The time of treatment is 5 to 15 minutes.

The bath converts the residual silver halide in both layers into silver ferrocyanide without affecting the first developed silver images.

The next step in the processing is the toning of the silver ferrocyanide, that is the conversion of said body into colored metallic compounds or salts, a different compound being produced in the two layers.

In accordance with the present invention this step is performed in a mixed toning or conversion bath such as the following:

|    |                              |     |
|----|------------------------------|-----|
| 5  | <i>Formula III</i>           | cc. |
| 25 | 10% ferric nitrate solution  | 1   |
|    | 10% uranium nitrate solution | 4   |
|    | 10% nitric acid              | 5   |
|    | 10% potassium bromide        | 2   |
|    | Water to                     | 50  |

30 The exact proportions of the components in this bath will depend on the thickness of the gelatine layers and the characteristics of the gelatine used, and the above formula is accordingly given as an indication of the proportions which might be necessary. The time of immersion in the bath for this method of working is not critical and may be varied from 10 minutes to 30 minutes for optimum results.

40 The ferric nitrate converts the silver ferrocyanide to Prussian blue and the uranium nitrate converts the silver ferrocyanide to uranyl ferrocyanide which is of red color. It has been found that such a bath can be caused to deposit the Prussian blue for a predetermined depth only

45 below which the uranyl ferrocyanide is deposited, enabling the Prussian blue to be deposited exclusively in the surface stratum or layer while the uranyl ferrocyanide lies immediately below. No full explanation of this phenomenon can be

50 given; it is considered however that in the course of penetration into the layers the ferric salt takes precedence as it gives Prussian blue which is less soluble than the uranyl ferrocyanide. The uranium nitrate is itself a tanning agent and 55 hardens the gelatine of the emulsion as it penetrates and this prevents the ferric salt from penetrating into the gelatine, thus limiting the zone of penetration of the ferric salt while below the uranium salt is effective for the formation of the red image.

60 It is noticeable however that the proportion of potassium bromide in the bath exerts a considerable effect on the relative deposits of the two toned salts; decrease in the proportion of bromide tending to reduce the proportion of uranyl ferrocyanide to Prussian blue while an increase limits the depth of blue and increases the depth of the red. Any acceptor for silver ions could be used in place of potassium bromide.

65 The applicant is unable to offer any explanation as to this phenomenon and directs attention to the fact that the production of a deposit of Prussian blue at any particular point of the upper layer or stratum is not necessary to prevent the zone of formation of the Prussian blue from 70 extending to any greater depth than is required.

for the image it records, that is to say the zone of formation of the Prussian blue can be caused to occupy a given depth of the emulsion layers while immediately below lies the zone of formation of the uranyl ferrocyanide, irrespective of the quantities of either which are deposited at any one point.

It will be appreciated that the formula given above may have to be modified according to the characteristics of the material under treatment and also the thickness of the layers in order to obtain the desired result namely that a blue image is produced in the surface layer and a red image in the under layer.

The final step, apart from whatever washing operations are necessary during and after processing is the removal of the first developed silver and of any unaffected silver salts with a suitable reagent such as Farmer's reducer, leaving a reversed color image which correctly reproduces the colors of the original subject within the limitations of the two-color process. As it is desirable for the stability of the toned images that the reducer should be acid, and as Farmer's reducer cannot be made up with hypo containing the customary potassium matabisulphite it has been found convenient to adopt the following:

|                 |      |     |
|-----------------|------|-----|
| A. Hypo         | gms. | 80  |
| Sodium acetate  | gms. | 4   |
| 10% acetic acid | ccs. | 4   |
| Water to        | ccs. | 400 |

B. 10% potassium ferricyanide.

For use add 1 part B to 3 or 4 parts A.

If the material includes a transparent layer 35 containing zinc hydroxide as referred to above, this is converted to an opaque white layer during the processing, either at a separate stage, or by the action of one of the processing baths. For example the first developer will normally contain sodium carbonate and this may convert the zinc hydroxide into white zinc carbonate. Alternatively the potassium ferrocyanide in the ferrocyanide conversion bath (Formula II) may convert the zinc hydroxide into white zinc ferrocyanide. Alternatively a separate bath of sodium carbonate or potassium ferrocyanide may be used at a suitable stage of the operations.

Where the material incorporates a stripping layer, at the completion of the processing, the material is treated according to the nature of the stripping layer in such manner, as by immersion in warm water, as to enable the colored image layers to be removed from the original support and transferred to a new support, for instance of paper.

If however the material is to be processed to form a colored original from which duplicate colored copies can be made, the colored image layers, processed as above described may be left on the original transparent support and copied onto a similar material by printing successively with differently colored printing lights or with white light or white light corrected by the interposition of corrective filters so as to have the desired 65 printing values. In this case, if the material includes a layer which can be rendered opaque white if desired, the material is so treated that this layer is unaffected.

Although the material has been described as 70 consisting of two superimposed photographic emulsion layers, a material could also be used consisting of a single orthochromatic emulsion layer part of the depth of which is sensitised by the controlled penetration of a sensitiser, that

5 is to say the layer is treated in a solution of a red or red-orange sensitising dye in alcohol for a sufficient period of time for the dyestuffs to penetrate to a limited depth and sensitise that part of the depth of the emulsion. Such sensitising dye bath preferably also contains a proportion of a filter dye which is such as to penetrate into the layers sufficiently to act as a filter dye to prevent the access of blue and green light into the sensitised stratum or depth of emulsion. Such filter dye may be an orange or red dye according to the characteristics of the sensitising dye used.

10 As specifically described the image produced in the under layer or stratum, consists of uranyl ferrocyanide. This gives a red image which is not altogether satisfactory and the present invention also provides a method of altering the color of such image by the application of a dye-toning dye which will mordant either to the uranyl ferrocyanide or to a conversion product derived therefrom.

15 In carrying this part of the invention into effect, the material, after processing to produce the Prussian blue and uranyl ferrocyanide images, is treated in a zinc salt conversion bath which converts the uranyl ferrocyanide into zinc ferrocyanide which is an effective mordant for many dye-toning dyes. Such a bath may contain:

Formula IV

|                             |     |    |
|-----------------------------|-----|----|
| Oxalic acid, 5%             | cc. | 5  |
| Zinc sulphate, 10% solution | cc. | 5  |
| Water to                    | cc. | 20 |

20 The toning dye may be added to this conversion bath or it may be used at a subsequent stage. A suitable dye is Rhodamine G which is made up to a 1/2% solution containing acetic acid up to a strength of about 1%. By reason of this treatment a dye-toned image of a satisfactory color can be formed in the under layer; this zinc salt bath has no effect on the already formed Prussian blue image in the top layer, nor does the dye solution become mordanted to said image. After the toning operation, excess dye is washed out, acidulated water being used if desirable, to leave a pure dye image. Obviously the replacement of the uranyl ferrocyanide image by a dyestuff image need not be complete unless desired.

25 The invention is also applicable to a three color picture and for this purpose a three layer material is preferably used although a single emulsion could be used of which the different strata are sensitised for different spectral regions. It is conceivable that a mixed toning bath could be used containing different toning compounds for the production of three color images and that by suitable selection of such compounds and of the other components in the treatment bath, such as the proportion of potassium bromide, the different color toning products would be formed or deposited in the different layers or strata.

30 Preferably however the procedure indicated above for the production of two differently colored images in two layers, is used for two of the colored images while the third image is produced by other means known in the art.

35 Various means may be used to obtain this third image and the third image layer could be coated on the opposite side of the material to the other two layers. In this way the one side of the material could be processed independently of the other by known flotation processes in which the

material is treated in a bath by floating over the surface thereof in such manner that the under side only is treated.

This procedure enables the third layer to be processed to form a color positive or negative image by dye toning, by color development, either with the color coupling component added to the emulsion at the time of manufacture or with the coupling component added to the developer, by the formation of a dyed gelatin relief image or by other similar processes. As an alternative to a flotation process, the layer or layers on one side may be protected from the action of a treatment bath used for the processing of the layers or layer on the other side, by means of a varnish coating of collodion, benzyl cellulose or the like. To permit the so-protected layer to be processed the protective layer may be removed by means of a suitable solvent for the varnish; thus acetone could be used for removal of a collodion varnish layer.

In one particularly convenient example all three layers are coated on one side of the support the layer nearest the support containing a proportion of a dye diffusely distributed therein which is capable of being selectively destroyed in the presence of and at the points occupied by a silver image to form a dye image, by the method commonly known as the silver dye-bleach process. This method is particularly applicable to the production of a natural color positive picture on the original exposure material or by copying from a natural color positive, since if the thiourea-ferrocyanide bath (Formula II above) is used for the production of silver ferrocyanide from the residual halide in all the layers, the same bath will perform the selective destruction of the diffuse dye in the bottom layer if a suitable dye is chosen. Many such dyes are known in the art and need not be listed here.

The material used for carrying this method into effect comprises a transparent support, conveniently of celluloid. On this is coated a non-color-sensitised silver halide emulsion which is diffusely dyed yellow with a suitable dye capable of being selectively destroyed in a thiourea bath or other suitable reagent. There is then coated a green sensitive emulsion followed by a red sensitive emulsion. There is no need to provide a yellow filter layer since the yellow-dyed bottom layer will perform the function of preventing access of blue light into the green and red sensitive layers; further if the green sensitive layer is insensitive to red and the red sensitive layer insensitive to green no filter layer whatever is necessary, giving a material which is of relatively simple construction. Clear gelatine layers can of course be provided between the emulsion layers if desirable to facilitate the subsequent processing. Further there may be interposed between the support and the lowermost emulsion, a stripping layer, or an initially transparent layer which can be rendered opaque white during the processing, as explained above in connection with the two-color process.

Such material is exposed through the base either in a camera to an original subject or in a printing machine for copying and the first step in the processing is the development of the latent images preferably in a silver solvent developer (Formula I above). Thereupon the unaffected silver halide in all three layers is converted to silver ferrocyanide, preferably without removal of the first developed silver, by means of a thiourea-ferrocyanide bath such as that given in

Formula II above. This bath may itself be of such character as to destroy selectively the yellow dye in the bottom layer at the points of the original silver image to form a positive yellow image in that layer. If necessary a separate dye-destruction bath could be used at any convenient stage of the processing.

Thereupon the material is treated in a mixed toning bath similar to that given in Formula III above but so constituted that the Prussian blue is deposited in the surface layer while the uranyl ferrocyanide is deposited below that while the silver ferrocyanide below that is substantially unaffected, probably on account of the tanning of the overlaying layers.

The material is now treated in a bath which removes the first developed silver images from all the layers as well as the silver ferrocyanide from the bottom layer and any remaining silver salts. Farmer's reducer can be conveniently used for this purpose or the alternative form above referred to. Finally the uranyl ferrocyanide may be converted to zinc ferrocyanide and the latter dye toned for instance with Rhodamine G as explained above (Formula IV) or the two baths combined.

This procedure enables a natural color picture to be produced on a multi-layer material of relatively simple construction and by a relatively simple processing technique. The picture obtained could be used as a transparency and the invention is of course applicable to kinematograph records. A print which can be viewed by reflection may be obtained by utilising the layer between the emulsion layers and the support which can be rendered opaque white at a suitable stage in the processing or by means of a stripping layer as above referred to which enables the colored layers to be transferred to a paper support.

It is also possible to produce a multi-color negative record, in which the layers are colored complementarily to the layer sensitivity or otherwise. In this case the latent images are developed in a negative developer, and then the layers are fixed and the developed silver converted by an oxidising bleach bath to silver ferrocyanide. The latter may then be toned in a mixed toning bath of the character of that given in Formula III so as to affect the silver ferrocyanide deposits in the two outer layers. With regard to the lowermost layer, this may be diffusely dyed during manufacture and the colored image therein produced by means of a reagent which is effective at the points unoccupied by silver so as to give a negative color image. Such a reagent may be effective only when the image is represented by silver and in that case, the production of the color image would be effected after development and fixation but before conversion of the silver into ferrocyanide.

I claim:

1. A method of producing a natural color photograph on a material including a transparent base, a blue sensitive emulsion layer on said base which layer is diffusely dyed yellow, and green and red sensitive emulsion layers coated on said blue sensitive layer, said red sensitive layer being outermost, comprising exposing said material to form latent images in the different layers, developing such latent images, converting the residual silver halide in said layers into silver ferrocyanide in a bath containing a ferrocyanide and a substance which renders the silver ferrocyanide less soluble than the silver halide, toning the

silver ferrocyanide in the green and red sensitive layers in a bath containing a ferric salt and a uranium salt to form a Prussian blue image in the red sensitive layer and a uranyl ferrocyanide image in the green sensitive layer, and at any stage selectively destroying the yellow dye in the blue sensitive layer at the points occupied by the developed latent image therein.

2. A method of producing a natural color photograph on a material including a transparent base, a layer thereon containing colloidal zinc hydroxide, a blue sensitive, yellow-dyed photographic emulsion layer and green and red sensitive emulsion layers, said red sensitive layer being outermost, comprising exposing such material through the base to form latent images in the three emulsion layers, developing such latent images, converting the residual silver halide in said layers into silver ferrocyanide without affecting the developed latent images, toning the silver ferrocyanide in the red and green sensitive layers into Prussian blue and uranyl ferrocyanide respectively in a bath containing a ferric salt and a uranium salt, selectively destroying the yellow dye in the blue sensitive layer to form a positive yellow image at any stage and converting the colloidal zinc hydroxide into an opaque white zinc salt.

3. A method of producing colored images in a material embodying an emulsion coat which is differently color-sensitive at different depths respectively comprising exposing such material to

5 produce latent images in said emulsion coat, developing such latent images, producing silver ferrocyanide images in the different depths of said coat, toning said silver ferrocyanide images in a bath containing a ferric salt and a uranium salt to form in one operation a surface image of Prussian blue and an image of uranyl ferrocyanide below that and dye-toning said uranyl ferrocyanide.

4. A method of producing colored images in a material embodying an emulsion coat which is differently color-sensitive at different depths respectively comprising exposing such material to

10 produce latent images in said emulsion coat, developing such latent images, producing silver ferrocyanide images in the different depths of said coat, toning said silver ferrocyanide images in a bath containing a ferric salt and a uranium salt to form a surface image of Prussian blue and an image of uranyl ferrocyanide below that, converting said uranyl ferrocyanide to a metallic salt which is a dye-mordant and treating the material in a dye-toning bath.

ALAN GILBERT TULL.